

# UNITED STATES PATENT OFFICE.

JOHN G. GOTTY, OF JACKSONVILLE, FLORIDA.

## PROCESS FOR LINING TURPENTINE-BARRELS.

1,323,528.

Specification of Letters Patent.

Patented Dec. 2, 1919.

No Drawing.

Application filed November 30, 1917. Serial No. 204,702.

*To all whom it may concern:*

Be it known that I, JOHN G. GOTTY, a subject of the King of Bavaria, residing at Jacksonville, in the county of Duval and State of Florida, have invented new and useful Improvements in Processes for Lining Turpentine-Barrels, of which the following is a specification.

The invention relates to a process for lining turpentine barrels or other vessels to prevent leaking, and relates also to a cementing process for closing leaks on the outside of said barrels and other vessels.

It is the common practice at the present time to apply a coating of glue on the inside of the turpentine barrels and, as this glue must be applied when hot, it does not effectively close all the pores and openings in the barrel. The barrels, therefore, must be subjected to several coats of glue to completely close all leaks and these several operations are expensive in the matter of labor, time and material.

The improved process consists in applying the lining coat of glue simultaneously with the tanning solution. The glue is dissolved in water to which there is added the tanning substance and some ammonia alum and strong vinegar or other acid, the proportion of water being enough to hold the composition in solution. The addition thereafter of a few drops of carbolic acid or some other disinfectant serves to prevent the glue from rotting. This preparation is then applied when cold and it impregnates the wood of which the barrels are made. After drying, the evaporation of a certain proportion of the water leaves the coating in a soft pliable state, as when the glue coating is covered with a tanning substance.

This preparation of the glue, together with the tanning solution and with the ammonia alum and vinegar or some other acid or disinfectant, as aforesaid, is useful for all purposes where glue is required.

The tanning substance mixed with the glue serves to make the latter more undissoluble, tight and durable, while the ammonia alum conserves the glue and in connection with the tanning substance keeps the glue in a more pliable state than would be the case were the tanning substance alone used.

In connection with this process, it is possible to convert the lining substance into a cement by the addition of enough ammonia alum to form a thin paste which may be applied on the outside of the barrel at points where leaks appear. This paste, after having been applied and when set and given a coating of ordinary paint, effectively closes any leak from the outside.

Having thus fully described this invention, what is claimed as new and useful, is:

1. The method of coating barrels and the like which consists in applying to a surface of a barrel a composition of glue and water to which there is added a tanning solution, some ammonia alum, some acid and some disinfectant.

2. The method of closing leaks in barrels and the like which consists in applying to a part of the surface of the barrel a cement composed of glue dissolved in water, a tanning solution and ammonia alum, and thereafter applying over the cement when set, a coating of paint.

In testimony whereof I affix my signature.

JOHN G. GOTTY.